

## UNITED STATES PATENT OFFICE.

MARY E. PENNINGTON, OF ST. DAVIDS, PENNSYLVANIA, AND ALEX BROOKING DAVIS,  
OF CINCINNATI, OHIO.

## MANUFACTURE OF STRAWBOARD.

No Drawing.

Application filed April 18, 1925. Serial No. 24,273.

For a long period of time strawboard has been manufactured by variations of a process which involves the disintegration of the straw by means of lime or soda, washing the resulting pulp and converting into board in the known manner. The resulting product contains compounds which are evidently volatile, since when used in the manufacture of containers for food products, for instance, the so-called "flats" and "fillers" for egg cases, the contents of the containers take on what is commonly called "the strawboard odor and taste," which is objectionable in many respects.

15 The principal object of our invention is to provide inodorous strawboard, and to provide strawboard which when used in the manufacture of containers for food products does not impart objectionable odor or 20 taste to the contents of the container; also to provide strawboard which is sterile.

Another object of our invention is to provide a process for producing such inodorous and sterile strawboard, and to provide a 25 process which is adapted to commercial use.

Other objects of our invention will be in part obvious and in part pointed out hereinafter.

We have found that if either raw straw 30 or disintegrated straw (pulp) is distilled with steam, the major portion or all of the volatile odorous compounds contained in the straw fibres may thereby be removed.

Straw is heavily contaminated with molds 35 and bacteria, especially of the spore-forming variety, and even distillation with steam may not destroy all of these organisms. Germination may produce bacteria which will react upon small amounts of carbohydrates and other organic constituents of the straw to produce odorous compounds, and it is, therefore, evident that a further improvement would be the complete sterilization of the straw or straw pulp at the time 40 the volatile constituents are removed. We have accomplished this by adding to the straw or straw pulp in the stills a quantity of sodium fluoride, which is highly toxic to bacteria and molds, and when a sufficient 45 concentration of this material is used, a sterile board results. No doubt, other disinfectants could be found which are suitable for the work, and we do not restrict ourselves to sodium fluoride. However, that

product was chosen as probably being lowest 55 in cost for the purpose and large amounts may be used since it is recoverable in the filtrate.

In distilling the straw or straw pulp with steam only sufficient steam need be passed through the material to remove the volatile compounds, and since they are volatile at ordinary temperatures as well as at the temperature of boiling water, it is evident that they are capable of being removed at temperatures below that of steam at atmospheric pressure. Therefore, the volatile compounds can be removed by the use of steam in an apparatus to which a fairly high 60 vacuum has been applied, with a resulting 65 saving in the amount of steam required and a reduced cost per ton of material treated.

The volatile compounds of straw impregnate all portions of the fibre, and steam distillation removes only that volatilized from 70 the outer surface of the fibre, but all is removed by continuing the distillation for a period, since the volatile odorous compounds are water soluble and apparently rapidly 75 diffuse out of the fibre or fibre cells. This 80 may be accelerated by first putting the straw fibres (raw straw or pulp) under steam pressure in a closed vessel, then quickly releasing the pressure, thereby breaking down the fibre or fibre cell walls and exposing the 85 volatile compounds contained to a more rapid volatilizing action.

After the removal of the major portion of the volatile odorous compounds by means of steam distillation, the small remaining 90 amount of volatile impurities may be removed or destroyed by means of ozonized air or the application of ozone to the mass in any known manner, the ozone in this case 95 replacing the use of sodium fluoride or other disinfectants.

After treatment the mass is filtered and made into board in the well known manner. The disinfectant may be recovered by evaporation of the filtrate.

Strawboard which has been deodorized is 100 applicable for packing many food products and the deodorized board may be used for the manufacture of numerous kinds of food cartons and packing cases. Furthermore, 105 sterile board or a board which is practically sterile should have many advantages over a non-sterile board for use in packing

products subject to the action of such molds and bacteria as are carried by the ordinary board.

Deodorized straw board pulp is suitable 5 for mixing with other odorless fibre pulp material for the manufacture of compounded pulp board, which will be practically non-odorous and suitable for the manufacture of cartons and cases for the packing of foods 10 and food products.

As many changes could be made in the above process, and many apparently widely different embodiments of the invention could be made without departing from the scope 15 thereof, it is intended that all matter contained in the above description be interpreted as illustrative and not in a limiting sense.

It is to be understood that the term "straw fibre" as used in the above description and 20 in the appended claims refers to straw fibre in raw straw and also to straw fibre in disintegrated straw and in straw pulp.

What we claim is:—

1. Strawboard comprising disintegrated 25 new straw disinfected and steam distilled, the strawboard being inodorous and sterile.

2. As a new product suitable for the manufacture of food cartons and parts thereof, inodorous and sterile strawboard pulp comprising new straw disintegrated, disinfected 30 and steam distilled.

3. As a new product suitable for the manufacture of food cartons and parts thereof, inodorous and sterile strawboard pulp comprising new straw disintegrated, disinfected and steam distilled, and containing traces of 35 a disinfectant.

4. As a new product suitable for food cartons and parts thereof, inodorous and sterile strawboard comprising new straw disintegrated, disinfected and steam distilled, and containing traces of a disinfectant. 40

5. As a new product suitable for the manufacture of food cartons and parts thereof, inodorous and sterile strawboard pulp comprising new straw disintegrated, disinfected and steam distilled, and containing traces of 45 sodium fluoride.

6. As a new product suitable for food cartons and parts thereof, inodorous and sterile strawboard comprising new straw disintegrated, disinfected and steam distilled, and containing traces of sodium fluoride. 50

7. The process of manufacturing material 55 suitable for food cartons and parts thereof,

which includes subjecting disintegrated new straw to the action of live steam in the presence of a disinfectant to render the same inodorous and sterile.

8. The process of manufacturing materials 60 suitable for food cartons and parts thereof, which includes rendering disintegrated new straw inodorous and sterile by distilling out by means of steam the volatile odorous principles in the presence of a disinfectant. 65

9. The process of manufacturing material suitable for food cartons and parts thereof, which includes removing from disintegrated new straw the volatile odorous principles by 70 the application thereto of steam in the presence of a disinfectant and permitting a portion of the disinfectant to remain to maintain sterility.

10. The process of manufacturing materials suitable for food cartons and parts thereof, which includes rendering disintegrated new straw inodorous and sterile by 75 distilling out by means of steam the volatile odorous principles in the presence of a disinfectant, the distillation being carried out at 80 sub-normal pressure.

11. The process of deodorizing straw fibre, which includes distilling straw fibre with steam and under sub-atmospheric pressure. 85

12. The process of manufacturing deodorized straw fibre, which includes distilling straw fibre with steam with which is mixed a quantity of ozonized air.

13. The process of deodorizing straw fibre, 90 which includes distilling out the volatile compounds with steam containing a quantity of ozone.

14. The process of deodorizing and sterilizing straw fibre, which includes distilling straw fibre with steam in the presence of 95 sodium fluoride.

15. The process of deodorizing straw fibre, which includes distilling out the volatile compounds with steam, and accelerating the treatment by placing the straw fibre under pressure and then suddenly releasing the 100 pressure.

This specification signed this 11th day of April, 1925.

MARY E. PENNINGTON.

This specification signed this 14th day of April, 1925.

ALEX BROOKING DAVIS.